

Dec. 24, 1957

1957 J. N. J. LEEMAN ET AL 2,817,441  
PROCESS FOR SEPARATING MIXTURE OF SOLID PARTICLES INTO  
FRACTIONS BY MEANS OF A HYDROCYCLONE  
Filed June 9, 1953

Filed June 9, 1953



FIG. I



FIG.2

## Inventors

Jan N. J. Leeman

Freerk J. Fontein

By Cushman, Darby & Cushman

ATTORNEYS

1

2,817,441

## PROCESS FOR SEPARATING MIXTURE OF SOLID PARTICLES INTO FRACTIONS BY MEANS OF A HYDROCYCLONE

Jan. N. J. Leeman, Brunssum, and Freerk J. Fontein, Heerlen, Netherlands, assignors to Stamicarbon N. V., Heerlen, Netherlands

Application June 9, 1953, Serial No. 360,464

Claims priority, application Netherlands March 2, 1953

7-Claims. (Cl. 209—211)

The present invention relates to a method for separating mixtures of solid particles into fractions by means of a hydrocyclone.

The term "hydrocyclone" as used in this specification and the claims hereof designates apparatus known per se comprising a chamber which is peripherally bounded by a smooth surface of revolution (by which we mean a surface generated by the rotation of a straight or a curved line about an axis) and tapering towards one end, the apparatus including one or more feed passages leading substantially tangentially into the chamber near the wider end thereof and two axial discharge apertures, viz., one at the apex of the chamber and hereinafter called "the apex aperture" and one in the wider end of the chamber and hereinafter called "the overflow aperture." The chamber may comprise conjoined cylindrical and conical portions and the tapering wall may conform to the wall of a true cone or may be slightly curved to present a concave or convex surface to the inside of the chamber. The overflow aperture may be and preferably is defined by a short conduit, hereinafter called "a vortex finder" extending axially into the wider end of the chamber. The dimensions of a hydrocyclone and the diameters of the feed apertures and outlets are such that, when a liquid is continuously introduced into the feed conduit(s) at a sufficiently high pressure, a rotary current is generated in the chamber, which current has an inner vortex directed towards the vortex finder, and another vortex around the first one, which moves axially in the opposite direction. Within the inner vortex there is an air core, provided there is no back pressure on the outlets. The chamber which generally is substantially conical, preferably has a mean angle of taper of from 5° to 30°, but angles up to 90° also have been successfully employed.

It is old to use hydrocyclones for the separation of solid particles according to grain size (classification) and for separation according to specific gravity (washing).

If a mixture of solid particles is to be classified the mixture is fed continuously under pressure into a hydrocyclone of suitable dimensions, together with a liquid whose specific gravity is lower than that of the particles to be classified. The fraction which then leaves the hydrocyclone continuously through the apex aperture contains substantially all the big particles and a small portion of the small particles, the fraction leaving the hydrocyclone continuously through the overflow aperture containing the main portion of the small particles.

If a mixture of solid particles is to be separated according to a certain specific gravity of separation, the mixture is fed continuously under pressure into a hydrocyclone of suitable dimensions, together with a liquid separating medium as hereinafter defined. The fraction which then leaves the hydrocyclone continuously through the apex aperture contains substantially only particles the specific gravity of which is higher than the specific gravity of separation together with separating medium, the fraction continuously leaving the hydrocyclone through the overflow aperture containing substantially all particles with a spe-

2

cific gravity lower than the specific gravity of separation together with separating medium.

The expression "liquid separating medium" as used above means an entirely liquid medium having an intermediate specific gravity, i. e., a specific gravity which is higher than the specific gravity of the specifically light particles and lower than the specific gravity of the specifically heavy particles constituting the fractions to be separated, or a medium comprising a liquid with solid particles considerably smaller than the particles to be separated in suspension, and having an intermediate specific gravity as aforesaid at a concentration of the suspension particles of fifty percent or less.

The suspension particles utilized in a separating medium of the second of the aforesaid kinds, are generally smaller than 200 microns and are often of a size of 60 microns or less, depending on the size of the particles to be separated, the specific gravity of the particles in the suspension and the conditions under which the separation takes place.

In carrying out the hydrocyclonic method of separation, especially if large hydrocyclones are used, the energy consumption is at present rather high. For example for a hydrocyclone with a diameter of 1,000 mm. it is necessary to employ a feed pressure corresponding to about a head of 12 m. of separating medium, and larger hydrocyclones require still higher pressures. In general the feed pressure should amount to the pressure exerted by a column of feed which has a height of six times the axial length of the hydrocyclone.

If the feed pressure is too low, the above mentioned hollow air core is not formed and the separation is not sufficiently accurate, in particular when large hydrocyclones, for instance with a largest diameter of more than 350 mm. are used. In washing operations, specifically light particles then get into the apex fraction, while, in classification at varying loads, too many fine particles enter the apex fraction of the hydrocyclone. Therefore it is usual to feed the separating medium together with the mixture to be separated into the hydrocyclone under considerable pressure by means of a pump. The use of pumps to this end is accompanied, however, with serious drawbacks, viz. the risk of blockage and of breaking up of the particles to be separated. A pump furthermore consumes much energy.

Now it is the object of the present invention to provide a method of operating a hydrocyclone wherein the pressure used is significantly below the pressure hitherto required but wherein satisfactory results in washing and classification are obtained. It is in particular the object of this invention to provide such method wherein the hydrocyclone is fed from a container, which may be a wash box the liquid level in which is less than six times the axial length of the hydrocyclone above the feed aperture of the hydrocyclone, without use being made of a pump. It is furthermore an object of this invention to operate a hydrocyclone with an axial length in the range from 0.7 to 9 m. with a feed head in the range from 0.4 to 5.7 times the axial length.

To attain these objects, according to the invention, the hydrocyclone is mounted in such a way that its axis makes a considerable angle with the vertical. Preferably the axis should be arranged either horizontally or so that the lowest generatrix of the hydrocyclone is substantially horizontal, or in an intermediary position.

We have found that with a hydrocyclone in such inclined position the desired sharpness of separation can be obtained at a much lower pressure than hitherto was necessary. The rapidly rotating current which is generated in a hydrocyclone when a high feed pressure is employed, gives rise to centrifugal forces which are much greater than the force of gravity, so that the posi-

tion of a hydrocyclone operated at high pressure generally is of secondary importance. Nevertheless hydrocyclones used in classification and washing have previously been operated with their axis substantially vertical, the apex pointing downwards, and with feed pressures corresponding with a feed head of at least six times the axial length of the hydrocyclone.

The invention is based on the discovery that the reason why big hydrocyclones which are positioned vertical need a comparatively high feed pressure is that, owing to their great length, these hydrocyclones contain such a tall liquid column that gravity becomes an important factor and influences the operation of the hydrocyclone. If, however, the hydrocyclone is given a sufficient tilt this phenomenon cannot occur.

In washing there is no air core if the feed pressure is too low and the hydrocyclone is positioned vertical. In that case specifically light particles may reach the apex aperture of the hydrocyclone, moving along the axis. If the hydrocyclone is tilted sufficiently there is an air core generally, and the specifically light particles cannot reach the apex aperture. Besides, if the hydrocyclone is positioned horizontal, there is no component of the gravitational force which can move the specifically light particles in the direction of the apex aperture.

If, in classifying, there is no air core, much liquid laden with fine particles leaves through the apex aperture, unless this aperture be chosen very small and its size be varied whenever there is a change in the composition of the feed. The latter demand is hard to meet in practice. If the hydrocyclone is tilted sufficiently an air core is formed, however, and the apex fraction will always have a high concentration, so that practically only the coarse particles leave the hydrocyclone through the apex aperture.

It stands to reason that the shape and the dimensions of the hydrocyclone moreover have to satisfy demands known in themselves; e. g., in general the discharge and feed apertures must be smaller than the overflow aperture.

With a vertical hydrocyclone the feed pressure ( $H$ ) (expressed in metres of separating medium) has to be at least about 6 times the axial length ( $L$ ) of the hydrocyclone. Now it has appeared that, if the axis of the hydrocyclone makes an angle  $\alpha$  with the vertical, the feed pressure need be only 6 times  $L \cos \alpha$ , or, expressed in a formula,  $\frac{1}{6} H$  equal to or greater than the absolute value of  $L \cos \alpha$ . However, this is of importance only if  $L > \frac{1}{6} H$ , because in the case that  $L < \frac{1}{6} H$  the axis of hydrocyclone may also be vertical.

According to one preferred mode of realising the invention the hydrocyclone is put with its axis substantially horizontal ( $\alpha$  about  $90^\circ$ ). The influence of gravity is then as small as possible and the ratio of  $\frac{1}{6} H$  to  $L \cos \alpha$  is infinitely large. It goes without saying that under those circumstances  $H$  cannot be made arbitrarily small, but must be great enough so that a rotary current is generated in the hydrocyclone.

A special advantage of a hydrocyclone which is positioned more or less horizontal is that, when this cyclone is fed from a tank situated higher than the cyclone, the feed conduit to the hydrocyclone may be straight. The feed conduit to a vertically arranged hydrocyclone usually has a bend in practice, which causes wear.

According to another preferred mode of realisation a conical hydrocyclone is so positioned that  $90 - \alpha$  is substantially equal to half of the apex angle and that the apex of the hydrocyclone is lower than its overflow aperture. This position offers the advantage that all the liquid can flow out of the hydrocyclone, which is of importance in case of shut-down and revision.

In order that the hydrocyclone may operate well it is furthermore desirable that the liquid which has been discharged through the vortex finder cannot flow back

to the vortex finder, as otherwise fine or specifically light particles might move to the apex aperture through the core of the cyclone and enter the apex fraction. In practice this involves, that the vortex finder must not discharge into a back-pressure chamber.

The invention, which is especially suitable for making separations by means of hydrocyclones having an axial length between 0.7 and 9 m. with a feed head in the range from 0.4 to 5.7 times the axial length of the hydrocyclone will be further explained with the help of the drawings.

Figure 1 is a section through a hydrocyclone which is so positioned that the lowest generatrix is horizontal.

Figure 2 is a view of a washing apparatus comprising a deep wash box and a hydrocyclone with its axis positioned horizontal.

In Figure 1, 1 is a hydrocyclone, consisting of a cylindrical section 2 and a conical section 3. The feed conduit 4 discharges tangentially into the cylindrical section 2 through the feed aperture 5, the cylindrical section being 20 closed by a plate 6 in which the vortex finder finder 7 is provided. The conical section 3 is provided with an apex aperture 8. The hydrocyclone is fed from the feeder tank 21. The level of the liquid in this tank is at a height  $H$  above the feed aperture 5. The axial length 25 of the hydrocyclone is denoted by  $L$ , the angle between the axis of the hydrocyclone and the vertical by  $\alpha$ .

The hydrocyclone 1 is mounted on a horizontal floor 10 by means of supports 9 and in such a manner that the lowest generatrix of the conical section 3 is horizontal, or 30  $90 - \alpha$  = half the apex angle of the hydrocyclone. 11 is a collecting tank for the light fraction discharged through the vortex finder 7 and 12 is a collecting tank for the heavy fraction discharged through the apex aperture 8. The collecting tank 11 is so constructed that the fraction 35 removed through vortex finder 7 cannot flow back to pipe 7.

#### Example 1

Different samples of raw bituminous coal having particle sizes ranging from 0.5 to 10 mm., from Staatsmijn 40 Emma, were washed in a conical hydrocyclone of the following dimensions:

|                                     |         |      |
|-------------------------------------|---------|------|
| Axial length of hydrocyclone        | mm      | 1210 |
| Diameter of the cylindrical section | mm      | 500  |
| Length of the cylindrical section   | mm      | 215  |
| Diameter of the feed aperture       | mm      | 100  |
| Diameter of the vortex finder       | mm      | 215  |
| Length of the vortex finder         | mm      | 215  |
| Diameter of the apex aperture       | mm      | 150  |
| Apex angle                          | degrees | 20   |

In the tests 1, 2 and 3 the axis of the hydrocyclone made an angle of  $80^\circ$  and in the tests 4 and 5 an angle of  $75^\circ$  with the vertical, so that the apex aperture was lower than the overflow aperture.

55 The feed took place from a tank the liquid level in which was 4.5 m. above the feed aperture. The separating suspension consisted of water and magnetite, 95% by weight of which magnetite was smaller than  $50 \mu$ .

The capacity amounted to about  $120 \text{ m}^3$  per hour. 60 The following results were measured:

| Test Nr.                        | 1     | 2     | 3    | 4     | 5     |
|---------------------------------|-------|-------|------|-------|-------|
| Heavy fraction (tons/hour)      | 6.9   | 15.5  | 5.6  | 17.3  | 6.9   |
| Light fraction (tons/hour)      | 23.8  | 20.6  | 19.8 | 20.3  | 22.0  |
| Spec. grav. suspension          | 1.505 | 1.505 | 1.51 | 1.50  | 1.50  |
| Spec. gravity of separation     | 1.64  | 1.63  | 1.67 | 1.59  | 1.63  |
| Enclosed area                   |       |       |      |       |       |
| Tromp curve (cm. <sup>2</sup> ) | 16    | 18    | 16   | 11    | 11    |
| Probable deflection             |       |       |      |       |       |
| (écart probable)                | 0.03  | 0.025 | 0.02 | 0.015 | 0.015 |

(For the meaning of "enclosed area Tromp curve" and "probable deflection" or "écart probable" see e. g. Coll. Eng. 1950, pp. 128-130 and 159, Cheradame and others).

Such good results cannot be obtained with the hydrocyclone in the vertical position.

## Example 2

Raw coal fines were washed in a conical hydrocyclone of the following dimensions:

|                                     |                 |        |
|-------------------------------------|-----------------|--------|
| Axial length of the hydrocyclone    | mm              | 1780   |
| Diameter of the cylindrical section | mm              | 700    |
| Length of the cylindrical section   | mm              | 420    |
| Feed aperture                       | mm <sup>2</sup> | 86×176 |
| Diameter of the vortex finder       | mm              | 300    |
| Length of the vortex finder         | mm              | 420    |
| Diameter of the apex aperture       | mm              | 220    |
| Apex angle                          | degrees         | 20     |

The axis of the hydrocyclone was horizontal and the hydrocyclone was fed from a tank situated at a height of 5.90 m. above the cyclone. The separating suspension had a specific gravity of 1.53 and consisted of water and magnetite, 95% by weight of which was smaller than 50 $\mu$ .

The feed contained a large percentage of slush, owing to which the viscosity of the suspension was high, which had an unfavourable influence on the result. The enclosed area of the Tromp curve of the particles of 1-2 mm. was 62 cm.<sup>2</sup> and the probable deflection amounted to 0.08, which, under the given conditions may be called very good.

## Example 3

A mixture of sand and loess in water was classified in a conical hydrocyclone of the following dimensions:

|                                     |         |     |
|-------------------------------------|---------|-----|
| Axial length of the hydrocyclone    | mm      | 945 |
| Diameter of the cylindrical section | mm      | 350 |
| Length of the cylindrical section   | mm      | 150 |
| Diameter of the feed aperture       | mm      | 70  |
| Diameter of the vortex finder       | mm      | 230 |
| Length of the vortex finder         | mm      | 150 |
| Diameter of the apex aperture       | mm      | 70  |
| Apex angle                          | degrees | 20  |

The hydrocyclone was so positioned that its axis was horizontal and it was fed from a tank situated at a height of 3 m. above the cyclone. Under these conditions its capacity amounted to 53.3 m.<sup>3</sup> per hour.

The suspension contained 50 grams of solid material per litre. The grain distribution in the feed and the results of the classification appear from the following table:

| Grain size (in $\mu$ ) | Percent of total in feed | Percent of grain fraction in discharge fraction |
|------------------------|--------------------------|-------------------------------------------------|
| +350                   | 0.08                     | 100                                             |
| -350+210               | 2.96                     | 100                                             |
| -210+105               | 18.21                    | 100                                             |
| -105+75                | 4.96                     | 99                                              |
| -75+50                 | 4.47                     | 95                                              |
| -50+40                 | 15.76                    | 34                                              |
| -40+30                 | 7.49                     | 19                                              |
| -30+20                 | 18.07                    | 2                                               |
| -20                    | 28.00                    | 0                                               |
|                        | 100.00                   |                                                 |

With the same hydrocyclone in the vertical position the classification is considerably worse at the same feed pressure and more fine particles get into the discharge fraction.

Fig. 2 shows a diagram of an attractive application of the invention. Here the feed conduit of the horizontal hydrocyclone 13 is directly coupled, via valve 14, to the short discharge pipe 15 of the deep wash box 16.

The column of suspension from the feed aperture of hydrocyclone 13 to the overflow trough 17 of wash box 16 provides the feed pressure H.

The mixture to be separated, e. g. raw coal, is introduced into the wash box at 18. The coal fraction is removed through the overflow trough 17, the shales and middlings through the discharge pipe 15. The latter fraction is subsequently separated in hydrocyclone 13 into a waste fraction, caught in the collecting tank 19, and a fraction consisting of middlings, caught in collecting tank 20. When operating in this manner the amount of energy required to make the separation between the waste and the middlings is very small.

We claim:

1. A process of separating a mixture of solid particles into fractions, which comprises the steps of continuously feeding the mixture together with a liquid medium under pressure tangentially into a hydrocyclone having an axial length of at least 0.7 metre, whereby separated fractions are discharged from axial overflow and apex apertures at opposite ends of said hydrocyclone, the axis of said hydrocyclone being inclined relative to the vertical at a considerable angle, and adjusting the feed pressure of said mixture and medium to a value, expressed in head of feed, substantially less than six times the axial length of said hydrocyclone but large enough to maintain a central air column in said hydrocyclone.
2. Process according to claim 1, in which the hydrocyclone axis is horizontal.
3. Process according to claim 1, in which said hydrocyclone is conical and the angle of inclination between the hydrocyclone axis and the horizontal is substantially equal to one-half the apex angle of the hydrocyclone.
4. Process according to claim 1, in which the discharge fraction from the overflow aperture is prevented from re-entering the hydrocyclone.
5. Process according to claim 1, in which the discharge fraction from the apex aperture of the hydrocyclone discharges into air.
- 40 6. Process according to claim 1, in which the hydrocyclone is fed by the static head of a wash box positioned directly thereabove.
- 50 7. A process of separating a mixture of solid particles into fractions, which comprises the steps of continuously feeding the mixture together with a liquid medium under pressure tangentially into a hydrocyclone having an axial length of at least 0.7 metres, whereby separated fractions are discharged from axial overflow and apex apertures at opposite ends of said hydrocyclone, the axis of said hydrocyclone being inclined relative to the vertical at a considerable angle, and adjusting the feed pressure of said mixture and medium to a value expressed in head of feed, within the range of from 0.4 to 5.7 times the axial length of the hydrocyclone.

## References Cited in the file of this patent

## UNITED STATES PATENTS

- 2,639,862 Watts May 26, 1953  
2,668,620 Fontein Feb. 9, 1954